

## UNITED STATES PATENT OFFICE

VALDEMAR WILLEMOËS D'OBRY, OF SCHLACHTENSEE, NEAR BERLIN, GERMANY

PROCESS FOR THE MANUFACTURE OF UNBLEACHED PAPER, CARDBOARD, AND THE  
LIKE

No Drawing. Application filed May 1, 1924, Serial No. 710,452, and in Germany May 25, 1923.

My invention relates to improvements in the manufacture of paper, cardboard and the like, and more particularly to a process for making paper, cardboard and similar pulp fabrics from dry grasses, reed-grasses, cereal-grasses and similar species of plants, and in particular corn straw. These materials in the claims for convenience are referred to as "grasses".

10 Essentially my new process consists in only steaming these plants and then breaking them up mechanically into fibres, whereupon the stuff thus produced may be directly worked into unbleached paper, cardboard, and the  
15 like.

My process is based upon the fact that by the treatment with steam at a certain pressure and during a certain period, not only a part 20 of the incrustations, but also the largest portion of the natural glutens or vegetable glues remain in the stuff together with the fibres and are not separated during the subsequent mechanical treatment in the presence of water, provided that washing is not too severe 25 during the mechanical process, or is omitted altogether. The natural glutens or vegetable glues are therefore contained in the stuff in such quantities that it is not necessary to add further quantities of glue in order to obtain 30 a good paper. The part of the incrustations which also remains in the stuff, serves as filling material.

Instead of adding sizing and filling materials to the pulp, as in the ordinary process of 35 paper manufacture, my simplified process produces a pulp or stuff, which is quite ready for the manufacture of unbleached paper, cardboard or the like without any addition of sizing or filling materials.

40 My improved process may be carried out in the following manner:

The dry raw material, for instance the straw of cereals, legumes, potatoes, grasses or reeds is cut into a chaff. The chaff, preferably after moistening, is introduced into a boiler and is steamed therein under pressure. The pressure amounts to 5-6 atmospheres, and the steaming period lasts about 2 to 4 hours, according to the raw material employed. The thus steamed material is intro-

duced into a rag-engine, an edge-mill or similar disintegrating or reducing apparatus, in which it is broken up into fibres in the presence of water up to the desired degree of fineness. During this treatment, the raw material may also be washed. The pulp or stuff thus produced may directly be conveyed to the paper machine and be worked into unbleached paper, cardboard or the like.

In carrying out the above process the temperature and pressure as above indicated are adapted to the particular character of the raw material while the material is steamed as distinguished from being boiled or treated with hot water so as to retain the natural vegetable 60 glues with the fibers, while most of the incrustations and cement substances are merely softened to a degree sufficient to permit them to be broken up easily by subsequent mechanical treatment.

The retention of the natural vegetable glues of the plants during the steaming operation results in these adhering to the fibers in the product resulting from the subsequent mechanical crushing with cold water in which 70 the glues are not soluble. As a result the final product contains so much glue that the pulp may be used to manufacture most solid papers and cardboards without any addition of glue whatever, while the retention of the 75 incrustations results in the pulp containing a natural filler.

Heretofore it has been proposed to remove the natural glues from wood, straw and the like by boiling or steaming and to separate 80 out or dissolve the incrustations by chemical treatment. My improved process is distinguished from these in that it seeks to retain the glue and the incrustations.

If the material is moistened or wetted prior 85 to the steaming, this has the advantage that the tendency of the material to spread is reduced to such an extent that the holding capacity of the steaming apparatus is considerably increased, and even doubled under certain circumstances. The wetting also leads to a uniformly good condition of the product 95 of steaming.

The pulp produced according to the improved process furthermore forms a suitable 100

half-stuff for the manufacture of bleached paper and cellulose. The product obtained by steaming and mechanical treatment is then subjected to a further chemical decomposition. This decomposition may be effected in the usual manner, for instance by boiling with caustic chemicals and subsequent bleaching with chloride of lime. For these purposes, my invention provides a process which may be carried out in uncivilized countries rich in plants of the described species by means of native labour, and which results in a half-stuff for the manufacture of bleached paper and cellulose. In order to obtain the half-stuff, the mechanical treatment is preferably carried only so far that the product consists of well washed raw fibres.

Preferably a sterilizing substance or agent may be added to the product, in order to prevent rotting during the storage or the transport.

This half-stuff can be pressed into bales, cakes or similar pieces (referred to as "shapes" in the claims for convenience) on the spot of occurrence of the grasses and the like, and is then easy to handle and to be transported, and enables a favourable utilization of the apparatus, as space and chemicals can be considerably saved. In pressing, the product may be given such a shape, that it may be conveniently charged into the boiler without further treatment, such as cleaning, pounding, ramming or other disintegration.

It will be understood that I do not limit myself to the exact details of the process, and that these may be modified within the ambit of my claims without departing from the spirit of my invention or sacrificing any of its advantages.

What I claim as my invention and desire to secure by Letters Patent is:

1. That process consisting in moistening a grass, steaming the moistened grass under pressure and preventing the escape of substantially all of the constituents of said grass, and then mechanically disintegrating the mass.

2. That process consisting in wetting vegetable matter, steaming the wet matter under pressure and preventing the escape of substantially all of the constituents of said matter, and then disintegrating the mass.

3. That process consisting in moistening vegetable matter, steaming the moistened matter under pressure of approximately five-six atmospheres, and preventing the escape of substantially all of the constituents of said matter, and then mechanically disintegrating the mass.

4. That process consisting in moistening a grass, steaming the moistened grass under pressure of approximately five-six atmospheres and preventing the escape of substantially all of the constituents of said grass, disintegrating the mass, decomposing the dis-

integrated mass, and finally bleaching the decomposed mass.

In testimony whereof I have affixed my signature.

VALDEMAR WILLEMOËS D'OBRY.

70

75

80

85

90

95

100

105

110

115

120

125

130